

No. 691,565.

Patented Jan. 21, 1902.

E. NORTON.

ART OF ROLLING METAL INGOTS INTO THIN PLATES OR SHEETS.

(Application filed July 1, 1901.)

(No Model.)

2 Sheets—Sheet 1.



WITNESSES:

F. B. Townsend

W. M. Monday

INVENTOR  
BY *Edwin Norton*  
Munday, Darts & Adcock  
ATTORNEYS

No. 691,565.

Patented Jan. 21, 1902.

E. NORTON,

## ART OF ROLLING METAL INGOTS INTO THIN PLATES OR SHEETS.

{Application filed July 1, 1901.}

(No. Model.)

2 Sheets—Sheet 2.



**WITNESSES:**

*F.B. Townsend*

H. W. Monday

*INVENTOR.*

INVENTOR  
Edwin Norton  
BY

BY  
unday, Evans & ~~Adcock~~  
ATTORNEYS

# UNITED STATES PATENT OFFICE.

EDWIN NORTON, OF NEW YORK, N. Y., ASSIGNOR TO AMERICAN CAN COMPANY, OF JERSEY CITY, NEW JERSEY, A CORPORATION OF NEW JERSEY.

## ART OF ROLLING METAL INGOTS INTO THIN PLATES OR SHEETS.

SPECIFICATION forming part of Letters Patent No. 691,565, dated January 21, 1902.

Application filed July 1, 1901. Serial No. 66,659. (No specimens.)

*To all whom it may concern:*

Be it known that I, EDWIN NORTON, a citizen of the United States, residing in New York city, in the county of New York and State of New York, have invented a new and useful Improvement in the Art of Rolling Metal Ingots into Thin Plates or Sheets, of which the following is a specification.

This invention relates to improvements in the art, process, system, or method of rolling iron or steel ingots into plates or sheets for use in the manufacture of tin-plate or for other purposes.

Heretofore in the manufacture or rolling of thin sheets of iron or steel for tin-plate a metal ingot of any convenient weight and dimensions is first rolled into a bar-plate, ordinarily about eight inches wide and three-eighths of an inch in thickness and fifty feet more or less in length, according to the size of the ingot. In the most modern method this rolling of the ingot into the bar-plate is done at a single heat, but in many mills is done in two separate heats or steps. This bar-plate is then sheared transversely of its length into small bars, each about eight inches wide by, say, twenty inches long, for use in making, for example, twenty by twenty-eight inch tin-plate, which is one of the most customary sizes, the length into which the bars are cut corresponding to and varying with or dependent upon the width of "singles" or of the finished product produced therefrom. These small bars are then heated and separately rolled into small sheets, ordinarily called "singles," the same being in the case supposed, say, about twenty inches in width, net, (about one-fourth of an inch extra being allowed for trimming or cropping,) and about twenty-eight inches, net, in length, and about one-tenth of an inch in thickness, the rolling being done in the cross direction from that of the previous step or ingot-rolling—that is to say, in the direction of the smaller dimension of the bars. During this step, which may for convenience and sake of distinction be termed the "bar-rolling" or "breaking-down" step, two of the bars are always and necessarily handled together, heated together, rolled together, and kept continuously together, so that the bars will secure the same treatment, and thus when rolled out into singles be capable of being matched or superimposed without too extravagant waste in cropping or trimming. The singles thus produced are then matched or superimposed, reheated, and further rolled in "pairs" or "packs of two," this rolling being again done in the same direction of the length of the singles, so that the original length dimension of the bar which is the width dimension of the finished sheet designed to be produced in the case supposed may be continuously preserved. This step or rolling doubles the length of the singles, making that of the pair about fifty-six inches, net, or double the length of the finished product in the case supposed. The sheets or packs of two are then folded or doubled, reheated, and again rolled in "packs of four" or four thicknesses, the length being thus again drawn out to about fifty-six inches, net, and then the sheets are finally again doubled, reheated, and rolled in packs of eight or eight thicknesses until they are reduced to the required gage, the finished pack of eight being in the case supposed (that of making thin sheets twenty by twenty-eight) fifty-six inches in length, (net after trimming or squaring,) or double the length of the finished product, and twenty inches, net, in width. In this old method or process after the first step of rolling the ingot into the bar-plate the succeeding rolling steps all take place repeatedly in the same direction, all such rolling steps being continually in the direction of the width of the plate-bar after the initial rolling of the ingot into the plate-bar. This successive and continual rolling in the same direction injures the strength and quality of the metal and causes the finished product of thin sheets or plates produced to have too little coherence, strength, and tenacity except in a direction across the grain or fiber of the metal produced by the continuous rollings or drawings of the metal in one direction, and in this old method or process after the first step of rolling the ingot into the bar-plate all the numerous succeeding rolling steps involve the handling and the passing again and again between the

rolls of comparatively very small rolling units, amounts, or pieces of metal, the rolling unit being really the small bar about eight inches by twenty inches by three-eighths inch thick, though after the singles are produced from the small bar two of these singles are matched and handled together, being superimposed, and as substantially the same amount of time and labor is necessarily involved in the handling and repeatedly reheating and passing between the rolls this small eight by twenty by three-eighths bar unit as would be required for a much larger rolling unit this old system or method of rolling is slow, laborious, and expensive, and in addition to this, even in the most modern and economical of the old methods, the ingot is only reduced at its first or initial heat rolling step to a bar-plate about three-eighths inch in thickness, and the metal requires after being sheared into bars to be subjected to a separate reheating step before further rolling and before it is reduced to the thickness of the singles, which is about one-tenth of an inch, suitable for matching or superimposing and rolling in pairs or packs of two.

It is the object of the present invention to provide a simple, efficient, and practical process or method of rolling iron or steel ingots into thin plates or sheets, such as are required for use in the manufacture of tin-plate, by which these objections or difficulties may be obviated or overcome, by which a much better quality of thin sheets or plates may be produced in respect to ductility, strength, and toughness than is produced by the old methods, and by which much time and labor and cost of manufacture may be saved.

The present invention consists in the means or process employed to practically accomplish this important object or result—that is to say, it consists in the new process or method of rolling iron or steel ingots into thin plates or sheets of definite or required dimensions, comprising the following series or combination of successive steps:

First. Rolling the ingot, of any convenient weight and dimensions, into what may for sake of convenience and distinction be termed a "wide billet-bar" about twenty inches wide by about 1.808 inches in thickness and thirty or forty feet, more or less, in length, according to the weight and size of the ingot, the width dimensions being preferably one of the dimensions of the singles or of the finished product designed to be produced. (For convenience and clearness the process will be described, for example, as practiced in making tin-plate sheets of the particular size, twenty inches by twenty-eight inches, it of course being understood that for other sizes the figures or dimensions given will vary accordingly.)

Second. Cutting or shearing this wide billet-bar, while still retaining its initial heat, into billets or pieces twenty inches by twenty-eight inches by 1.808 inches, the length dimensions corresponding to one of the dimensions of the singles or of the finished product designed to be produced in the case supposed.

Third. Rolling these wide billets or pieces, while still retaining their initial heat, in the cross direction from that of the previous rolling—that is to say, in their twenty-inch direction—into thin bars, each, say, twenty-eight inches wide by eighty inches in length and by .45 inch in thickness, by passing the same back and forth between reversing-rolls, so that the rolling action upon the metal in this step is alternately in opposite directions.

Fourth. Continuing the rolling of these wide thin bars at the same initial heat and in the direction of their length into a long wide thin plate about twenty-eight inches wide by thirty-four feet in length and about one-tenth inch in thickness, which for convenience and distinction may be called "singles-plate." This final rolling action at the initial or first heat reduces the ingot to the thickness of the singles and is preferably performed by a continuous train of five stands of rolls.

Fifth. Shearing the wide thin singles-plate thus produced into singles ready to match, the same being each twenty inches, net, or twenty and one-fourth inches by twenty-eight inches by about one-tenth inch in thickness.

Sixth. Matching or superimposing the singles, reheating, and further rolling in pairs or packs of two in the cross direction from the last previous rolling—that is to say, in the direction of the length of the singles—thus extending the length of the pair to about fifty-six inches, net.

Seventh. Folding or doubling the pair, reheating, and again rolling in packs of four, thus again doubling the length to about fifty-six inches, net.

Eighth. Finally, again doubling, reheating, and rolling in packs of eight or eight thicknesses until the sheets are reduced to the required gage, their length being again doubled to about fifty-six inches, net, or twice the length of the finished product in the case supposed.

By this new or improved process it will thus be seen that the original ingot is reduced to the thickness of the singles, about one-tenth inch, at a single heat, the first or initial heat thus saving the time, labor, and expense incident to one reheating over the most modern and improved methods heretofore in use; also, that by the new process the direction of the rolling is changed or crossed twice instead of but once, as in the old process, in which all the rolling from the small bar, three-eighths inch thick, down to the finished gage takes place in the same direction without any crossing or alternation. For this reason the new process produces a greatly superior product in respect to ductility, strength, and toughness of the thin sheets, especially for withstanding folding or drawing strains at right angles to the direction of the last rolling, as the successive crossings of the direction of rolling tends to interweave the grain or fiber

produced by each successive cross-rolling, and by reason of the successive crossing or alternation of the direction of rolling the metal does not receive anything like the punishment, exhaustion, or strain that it does when the major portion of the rolling (from the small three-eighths-inch bar down to the thin gage required) takes place all in one direction, as in the old process, and by the new process also much annoyance, time, and labor is saved by reason of the fact that the small rolling unit (the eight-inch by twenty-inch by three-eighths-inch bar) is entirely dispensed with.

15 In the accompanying drawings, forming a part of this specification, to enable the invention to be more readily understood by those skilled in the art, I have illustrated in a conventional or diagrammatical manner at Figures 1 to 13 the ingot or metal being rolled in various successive steps or stages of the process, and at Fig. 14 have illustrated in a conventional or diagrammatic manner an apparatus, system, or arrangement of rolling-mills and machinery suitable for practicing the invention.

In the drawings, A, Fig. 1, represents the ingot of any suitable size—say twelve inches by twenty inches by four feet or more in length; B, Fig. 2, the wide billet-bar—say twenty inches by .8 inch by twenty, thirty, or forty feet in length; C, Fig. 3, the wide billet—say twenty inches by twenty-eight inches by 1.8 inches—into which the billet-bar is sheared or cut; D, Fig. 4, the wide plate (twenty-eight inches by eighty inches by .45 inches) into which the billets are rolled, in the cross direction from the last rolling by passing the same back and forth in opposite directions between reversing-rolls; E, Fig. 5, the wide singles-plate into which the wide plates D are rolled, (the same being, say, twenty-eight inches wide by thirty-four feet in length by one-tenth inch in thickness.) This represents the reduction at the first or initial heat of the metal.

F, Fig. 6, represents the singles into which the singles-plate is cut, the same being, say, twenty inches by twenty-eight inches by one-tenth inch; G, Fig. 7, a pair of the singles matched and reheated ready for further rolling in pairs or packs of two; K, Fig. 8, the pair reduced in thickness and doubled in length by rolling; L, Fig. 9, the pair doubled, reheated, and ready for rolling in packs of four; M, Fig. 10, the pack of four doubled in length and reduced in thickness by the next rolling; N, Fig. 11, the pack of four folded and doubled and reheated and ready for rolling in packs of eight; O, Fig. 12, the pack of eight rolled and extended in length, and P, Fig. 13, the finished sheet twenty inches by twenty-eight inches by 1.8 inch in thickness formed by cutting and trimming the pack of eight and separating the sheets thus formed.

65 The apparatus, conventionally or diagrammatically indicated in Fig. 14 as suitable for

use in practicing the process, comprises, preferably, a soaking-pit *a* for the ingots, a crane *b* for lifting the ingots onto the conveyer-table *c*, a four-high reversing rolling-mill *d*, 70 having, preferably, four horizontal and one or two pair of vertical rolls between which the ingot is passed back and forth until it is reduced to about 1.8 inches in thickness, a billet-bar-shearing mechanism *e*, having feed-table *f*, transverse conveyers *g g'*, a series of automatic reversing bar rolling-mills *h*, having each a feed-table *h'*, a continuous rolling-mill *k*, having, preferably, five stands of rolls arranged tandem, a rotary shear mechanism 80 *m* for shearing the singles-plate into singles, a series of rotary heating-furnaces *n* for heating the singles in pairs and packs of fours and eights, and a series of automatic finishing-mills for rolling the packs of twos and fours 85 and eights; and *q q' q''* indicate engines and *r r'* reversing-gear mechanisms for the ingot-mill *d* and the automatic reversing bar-mill *h*. Any other suitable kind or arrangement of mills and apparatus may, however, be used 90 in practicing the invention.

As in this invention the ingot is reduced at a single heat—the first or initial heat—to the thickness of the singles, and as the singles-plate thus produced at a single heat is 95 sheared into singles ready for matching, the singles are by this process produced of uniform size, weight, and dimensions, so that they match or superimpose accurately and without loss or waste of metal. In the processes heretofore in use where the singles are produced from separate small bars repeatedly rolled they always differ more or less in dimensions and thickness, however carefully they may be handled and heated to match together, and this causes a large waste of metal in trimming or cropping. By my process this loss or waste of material is almost entirely saved. After the singles are produced the successive reheatings and rollings in packs 100 of twos, fours, and eights are or may be the same as heretofore practiced.

The invention may also be used for manufacturing sheets or plates of various sizes and thicknesses. If thin sheets or plates are not 115 desired, one or more of the pack-rolling steps may be omitted.

I claim—

1. The process or method of rolling iron or steel ingots into finished product thin sheets 120 or plates of definite lengths and widths, suitable for tin-plate, consisting in first rolling the ingot into a long, wide billet-bar, then shearing such wide billet-bar into billets or bars whose length corresponds to one of the 125 dimensions of the singles or of the finished product to be produced, then rolling such wide billets or bars in the cross direction from the first rolling into a long, thin "singles-plate," then shearing the "singles-plate" into 130 "singles," then matching, reheating and rolling the "singles" successively in packs of

"twos" "fours" and "eights" in the cross direction from the last preceding rolling, substantially as specified.

2. The process or method of rolling iron or steel ingots into finished product thin sheets or plates of definite lengths and widths suitable for tin-plate, consisting in rolling the ingot, shearing it while hot into pieces corresponding in length to the length of the singles or of the finished product, cross-rolling such pieces into a long thin "singles-plate" without reheating, and then shearing the same into "singles" and matching, reheating and rolling in packs, substantially as specified.

15 3. The process herein described, consisting in the following successive steps, first rolling the ingot into a wide billet-bar; second, shearing it into wide billets or bars whose length corresponds to that of the "singles" or of the finished product; third, cross-rolling these wide billets or pieces in the direction of their width without reheating; fourth, continuing the rolling without reheating until the same is reduced to a long, wide "singles-plate;" 20 fifth, shearing the "singles-plate" into "singles;" sixth, matching, reheating and rolling in pairs or packs of two; seventh, folding or doubling the pair, reheating and rolling in packs of four; and, eighth, doubling, reheating and rolling in packs of eight, substantially as specified.

4. The process herein described, consisting in the following successive steps: first, rolling the ingot into a wide billet-bar whose width corresponds to the width of the "singles" or of the finished product to be produced; second, shearing it into wide billets or bars whose length corresponds to that of the "singles" or of the finished product; third, cross-rolling 35 these wide billets or pieces in the direction

of their width without reheating; fourth, continuing the rolling without reheating until the same is reduced to a long, wide "singles-plate;" fifth, shearing the "singles-plate" into "singles;" sixth, matching, reheating and 45 rolling in pairs or packs of two; seventh, folding or doubling the pair, reheating and rolling in packs of four; and, eighth, doubling, reheating and rolling in packs of eight, substantially as specified. 50

5. The process of rolling iron or steel ingots into thin sheets or plates of definite lengths and widths, consisting in first rolling the ingot in opposite directions by passing it back and forth between rolls into a billet-bar, then shearing it while hot into billets or bars corresponding in length to the length of the "singles" or of the finished product, then cross-rolling such billets or bars in opposite directions by passing them back and forth 55 between reversing rolls in the direction of their width, without reheating, and further rolling the same continuously into a long, thin "singles-plate" without reheating, and then shearing into "singles" and matching, 60 reheating and rolling in packs, substantially as specified.

6. The process or method of rolling iron or steel ingots into sheets or plates, consisting in first rolling the ingots, then shearing, then cross-rolling without reheating, then shearing into "singles" and then reheating and rolling in packs in the cross direction from the last preceding rolling, substantially as specified. 70

Dated June 26, 1901.

EDWIN NORTON.

Witnesses:

HENRY F. AKIN,  
T. S. WHEELER.